

April 30, 1946.

R. J. TAYLOR

**2,399,260**

## FILAMENTOUS PRODUCT

Filed June 8, 1943



Fig. 1.



Fig. 2.



Fig. 4.



Fig. 5.



Fig. 3.

BY

INVENTOR.  
ROBERT J. TAYLOR  
Carl A. Castellan  
ATTORNEY.

## UNITED STATES PATENT OFFICE

2,399,260

## FILAMENTOUS PRODUCT

Robert J. Taylor, Claymont, Del., assignor to  
American Viscose Corporation, Wilmington,  
Del., a corporation of Delaware

Application June 8, 1943, Serial No. 490,009

13 Claims. (CL 28—78)

This invention relates to filamentous or fibrous mats of extremely low density suitable for use as a heat insulation material, a buoyant material, for aerosol filtration, cushioning material and the like and to methods of producing them. The present invention is particularly a modification of the product and method disclosed in my prior applications Serial No. 479,889, filed March 20, 1943, and Serial No. 489,071, filed May 29, 1943.

Generally, the products of my prior applications are prepared by causing a bundle of continuous filaments to be fanned out under turbulent conditions into a filamentary sheet and to be wound in the form of a cylindrical band while the sheet as a whole is being waved or traversed either regularly or irregularly in a direction generally axially of the winding. After collection, the wound band is cut transversely and is then expanded by stretching in a direction transverse of the band while maintaining it taut along its length. The length of the band is somewhat reduced in the expansion process, but both the width and thickness are greatly increased to produce an exceptionally light-weight fibrous product. Products comprising hollow filaments have been produced in the same general procedure as disclosed in my later prior application.

In accordance with my present invention, products of the type disclosed in my prior applications are made from a mixture of different diameter filaments. As was pointed out in my prior application, products of this type are most satisfactory and have the most uniform texture as the result of thorough distribution of fibers in heterogeneous overlapping and interlacing relationship when made from filaments of finer diameters and especially when of diameters of the order of 10 microns or less. In accordance with the present invention, it has been found that the mats made from filaments of larger diameters can be greatly improved by incorporating a substantial proportion of comparatively small diameter filaments therein. The addition of the small diameter filaments not only improves the mat formation and its uniformity but also improves the cohesion and structural stability of the mat. In addition, by varying the proportion of small diameter filaments in the product, it is possible to control the air permeability of the fibrous mats produced therefrom, the greater the proportion of small diameter filaments, the lower the air permeability obtained.

Any method of combining the differently sized filaments together may be employed. Thus, the arrangement shown in Figure 15 of my earlier

5 prior application, in which one filamentary component coming from a suitable package thereof is fanned out just before it reaches the spinning bath in which the other component is freshly spun, may be used and is particularly advantageous when completely set filaments of large diameter are taken from an external package and fanned out into the spinning bath in which filaments of small diameter are being spun. Alternatively, separate spinnerets may be employed in a common spinning bath, one of the spinnerets being provided with differently sized holes or having the filamentary material pumped through it at a different rate so that different sized filaments are obtained from each spinneret. Again, 10 a single jet may be employed, some of the holes therein being distinctly larger than others therein. Again, a single spinneret may be employed where it is of the type in which separate spinning lines communicate with distinct orifices 15 therein. This may be accomplished by the arrangement of suitable partitions back of the spinneret face and arranging the connections to separate spinning lines so that one line communicates with certain compartments and the other line communicates only with the remaining compartments back of the spinneret face. Either the 20 same spinning solution may be pumped at different volumetric rates through the different lines and corresponding orifices in the spinneret or different filamentary material may be spun there-through, or, again, the orifices associated with one spinning line may be larger than those associated with the other spinning line. Where different filamentary spinning solutions are used, 25 one may be capable of producing hollow or inflated filaments of large diameter while the other may produce a fine diameter filament. In this modification, the orifices associated with each spinning line may be of the same size or different. Besides these methods of combining two filamentary materials, one or more filaments or twisted or untwisted bundles of filaments may be laid down with traverse about the wound filamentary band between the several convolutions 30 therein as it is being formed. Thus, a band of fine filamentary material may be collected upon a rotating take-up drum while additional filaments or yarns may be wound upon the drum at a different point of its periphery thus laying down the additional large filaments between the convolutions of the web-like sheet being collected 35 upon the drum.

40 The mats made in accordance with this invention may be of extremely low densities, this

45 50 55

characteristic being favorably influenced by the fact that large hollow filaments can be incorporated in large proportion. At the same time, in spite of the presence of the large diameter hollow filaments, the air and gas permeability is maintained low by virtue of the presence of the small diameter filaments intermingled and thoroughly distributed through the mats. As in my prior applications, the essential structure of the mat comprises criss-cross filaments lying substantially in generally parallel planes so that the mat is substantially laminar in character. By disposing the laminations substantially perpendicular to the direction of heat flow, it will be seen that there is no path provided by the mat for a direct heat conduction along solid filaments from the hot surface to the cold surface. The laminar character of the product assures that the travel of heat by conduction will be forced to take the longest possible route between the opposite faces of the mat. Mats of hydrophobic vinyl resins in particular exhibit moisture retentions of less than 0.05% at 58% relative humidity and 75° F., are highly resistant to attack by alkalis and mineral acids of all strengths, oils, fats, waxes, alcohols, etc., and are non-inflammable.

The filamentous masses of the present invention are characterized by a high resistance to transfer of heat by conduction as well as by convection, especially in the direction of their thickness. This is attributable to the extreme subdivision of the space occupied by the mats, by the criss-cross filaments extending in undulated planes substantially at right angles to the thickness of the mats and to the fact that the lattice work formed by the filaments in one web is out of alignment with that in adjacent webs lying generally parallel thereto. Each web appears to consist essentially of more or less filaments of various sizes intimately and intricately criss-crossed upon one another with, of course, considerable undulation and deviation from a flat plane. The superimposition of web on web of such irregularly arranged inter-crossing filaments with the additional waviness in the individual filaments produces a filamentous mass having an intricate network disposed across the path of travel in the direction of the thickness of the mat. All filaments in one web, lamination or strata do not contact all filaments in the next adjacent at the points where they appear to cross as a result of the distortion caused by the stretching. The result is a special network of filaments, none of which presents a solid path of conduction from one face to the other of the mat and across which the transfer of heat by conduction must take numerous lengthy deviations along the filaments lying at angles approaching a right angle to the path of heat transfer.

The various methods of combining the different size filaments and arrangements for executing the methods are illustrated by the following drawings, in which:

Figure 1 is an elevation view of one embodiment of the invention.

Figure 2 is a plan view of another arrangement for executing the invention.

Figure 3 is a cross-section showing one form of spinneret for simultaneously spinning filaments from material supplied through separate lines.

Figure 4 is an elevation showing another arrangement for executing the invention and

Figure 5 is an elevation showing a modification of the arrangement of Figure 4.

As shown in Figure 1, two spinnerets 2 and 3 are arranged one above the other and are supplied by separate feed lines. The filaments produced proceed through a common guide 4 having a flared mouth and a substantially cylindrical channel and then to a suitable take-up device 5 which may or may not be traversed as it is rotated. The take-up device may comprise a drum partially immersed in the coagulating bath and, as in my prior applications, the filaments are collected in the form of an annular band 6 comprising a number of superimposed convolutions each comprising a web-like sheet of the highly intercrossed and interlaced filaments.

One of the spinnerets shown in Figure 1 may be provided with larger size orifices and in such case, the spinneret supply lines may be connected to a common spinning pump from a single spinning line. Alternatively, the spinneret feed lines may be connected through separate pumps to a single supply line or through separate pumps to separate supply lines. Where the spinneret supply lines are connected through separate pumps to a common spinning solution supply line, the orifices in the spinnerets may be of the same size and the variation in size of filaments may be obtained by operating one of the pumps at a different volumetric rate than the other. Where the two spinnerets supply lines are connected through separate pumps to separate spinning solution lines, a distinct spinning solution may be supplied to each line, in which event, the arrangement lends itself very readily to the production of hollow filaments of large or small diameter from one of the spinnerets and fine filaments from the other. By any of these arrangements, the proportion of the number of fine diameter filaments relative to the total number of filaments may be varied as desired.

Figure 2 illustrates an arrangement in which a spinneret 7 (shown in greater detail in Figure 3) capable of spinning filaments from a plurality of separate supply lines (two, 8 and 9, being shown) is associated with suitable filamentary guides 10 and 11 and a suitable take-up drum 12 similar to that of Figure 1. The arrangement shown in Figure 3 for feeding separate solutions to separate orifices in the spinneret comprises a supply head 13 comprising two connections for the feed lines 8 and 9 and the spinneret proper 7, the space between the back face of the spinneret and the entrances 14 and 15 for the different spinning materials being partitioned transversely by a cylindrical disk 16 into a region immediately in front of the entrances 14 and 15 and another region immediately in back of the spinneret face. The former region is divided into two separate sections A and B by the partition 17. The latter region is divided by annular partitions 18 and 19 into concentric compartments C, C<sub>1</sub> and C<sub>2</sub> each of which are associated with one or more separate circles of spinneret holes. The section A is connected to compartment C<sub>1</sub> by suitable passages 20 in the disk 16 and the section B is connected to compartments C and C<sub>2</sub> by passages 21 and 22 respectively. It is obvious that the region immediately back of the spinneret face may be divided into any number of concentric compartments. The spinneret orifices associated with the several concentric compartments C, C<sub>1</sub> and C<sub>2</sub> back of the spinneret face may be of the same diameter or of different diameter and those associated with any given

compartment may comprise orifices of various diameters. The orifices may conveniently be arranged in circles of radii intermediate those of the annular partitions 18 and 19. This arrangement lends itself readily to the spinning of separate spinning materials or solutions and the production of filaments of different materials having either the same or different sizes or of the production of hollow filaments with solid filaments of the same or different spinning materials and either of the same or of different diameters.

In Figure 4, a spinneret 23 having orifices of the same size throughout is associated in a spinning bath with suitable guides 24 and 25 and a take-up device 26 which is partially immersed in the coagulating bath. The filaments proceeding from the spinneret may have any desired diameter and may advantageously be of relatively small diameter as compared to those which are to be wrapped upon the drum 26 in the following manner. Adjacent a portion of the periphery other than that at which the fine filaments proceeding from the spinneret 23 are received upon the take-up device or drum 26, other filaments, yarns or the like may be directed upon the winding by a suitable guide 27 which is traversed axially of the take-up device, the filaments, yarns and the like being supplied to the traverse guide from a suitable supply package 28, such as a bobbin, cake of rayon, and the like. While the traverse of the guide 27 may have any desired rate, it is preferred that it be controlled to such a rate that the helix angle of the yarn or filaments laid down upon the take-up device does not exceed about 10° and preferably is less, especially where a high proportion of filaments are to be combined with those spun from the spinneret in this manner.

Figure 5 is similar to Figure 4 but discloses an arrangement in which a plurality of separate 40 yarns, or twisted or untwisted bundles of filaments are supplied to the take-up drum 28 by means of separate traverse guides 27a, 27b, and 27c. The traverse guides are offset vertically so that their traverse motions do not interfere. The rate of traverse of the several guides may be the same or different, preferably the latter. In either of the embodiments of Figures 4 and 5, the take-up device 26 may be somewhat traversed axially or it may be rotated in fixed position.

#### Example

Two spinning solutions were extruded through separate groups of orifices in a spinneret of the type shown in Figures 2 and 3 into an aqueous sulfuric acid solution of 20% concentration. One of the solutions was formed in acetone of 8% by weight of a copolymer of vinyl acetate and vinyl chloride having a softening point 65 to 70° C., said copolymer having 90% by weight of vinyl chloride. The other solution comprised 10% of the same copolymer in acetone and about 2% of calcium carbonate. Spinning was performed with the coagulating bath at about 45° C. and the pump speeds and the speed of the take-up drum were adjusted so that the solid filaments had a diameter averaging 5 microns and the hollow filaments had a diameter of about 50 microns, the spinneret used being of the type shown in Figure 3 and being provided with concentric circles of holes, through 850 of which hollow filaments were produced and through 641 of which solid filaments were produced, the orifices yielding solid filaments being arranged in circles al-

ternating with those circles from which the hollow filaments were obtained.

After collection of the desired thickness of band, it was cut from the drum and stretched transversely of the general direction in which the filaments lie in the band to produce the expanded mat or bat of the type disclosed in my copending applications above referred to. In the final expanded bat, the hollow filaments were uniformly distributed among the solid filaments and the product exhibited an enhanced bulk as the result of the incorporation of the hollow filaments and improved structural stability as well as low air and water permeabilities which was imparted by the finer diameter filaments.

As in my copending applications, the products of this invention may be produced from any artificial continuous filaments, such as those of regenerated cellulose from viscose or cuprammonium cellulose, of cellulose organic derivatives, such as cellulose ethers and esters and particularly cellulose acetate, of vinyl resins, such as polyvinyl chloride, copolymers of vinyl chloride and vinyl acetate, after-chlorinated polyvinyl chloride, after-chlorinated copolymers of vinyl chloride and vinyl acetate and copolymers of vinyl chloride and acrylonitrile, or from any other material whether organic or inorganic, such as glass or mineral wool filaments. Natural continuous filaments, such as silk may also be used.

In addition, as disclosed in my prior application Serial No. 479,889, the product may be modified by subjecting the band before expanding it to shrinkage. Again, as suggested in that earlier application, the wound bands may be produced from a mixture of shrinkable filaments with non-shrinkable filaments or with a mixture of two or more types of filaments having different shrinkage characteristics. And, before expansion of the band, it may be subjected to a shrinkage agent which effects shrinkage of the more sensitive of the several materials of which the products are composed. Either the hollow filaments or the solid filaments, where products comprising a mixture of such are involved, may be more sensitive to shrinkage than the other type of filaments.

Another advantageous combination is obtained by mixing a minor proportion of potentially adhesive filaments with a relatively large proportion of filaments of non-adhesive material which, after collection upon the winding drum, may be subjected to an activating agent for the potentially adhesive filaments, such as heat, a solvent or swelling agent to render the potentially adhesive fibers tacky and to cause them to adhere to the nonadhesive filaments. In this case, either the hollow or solid filaments may be the potentially adhesive filaments.

Another variation involves the incorporation of filaments of a rubbery elasticity, such as rubber itself or any synthetic or substitute for rubber, for example a plasticized copolymer of vinyl chloride and vinyl acetate. The filaments of the rubber-like material may be of any diameter and may be combined in any proportion with the other filaments of the band, and the band, after cutting and removal from the take-up drum, exhibits a crinkled or corrugated surface. As a modification of this procedure, the rubber-like filaments may be incorporated within the band by means of the arrangement of Figures 4 and 5, the non-rubber-like filaments being produced from the spinneret and the rubber-like filaments being wrapped about the

convolutions thereof upon the drum under tension. After cutting the band, the rubber-like filaments contract and draw up the band to crinkle it. After expansion by stretching transversely of the length of the filaments therein, the crinkliness is converted into a puckered or pebbled effect of finer grained quality than that in the original band.

While preferred embodiments of the invention have been disclosed, it is to be understood that changes and variations may be made without departing from the spirit and scope of the invention as defined by the appended claims.

I claim:

1. A wound filamentous product comprising convolutions of a thin sheet of continuous filaments, the filaments in the convoluted sheet being irregularly disposed with respect to each other through the length of the convoluted sheet, the successive convolutions of the winding being haphazardly disposed with respect to each other, the filaments comprising a mixture of solid filaments having an average diameter between about 1 and 10 microns and hollow filaments having an average diameter of at least 10 microns.

2. A wound filamentous product comprising convolutions of a thin sheet of continuous filaments, the filaments in the convoluted sheet being irregularly disposed with respect to each other through the length of the convoluted sheet and comprising filaments having an average diameter between about 1 and 10 microns, the successive convolutions of the winding being haphazardly disposed with respect to each other, additional convolutions of hollow continuous filaments having an average diameter substantially larger than that of the first-mentioned continuous filaments and having their convolutions disposed between the convolutions of the sheet.

3. A low-density filamentous product comprising a bulky expanded mass of filaments exhibiting internal surfaces of cleavage, the strata comprising an irregular net work of intercrossing filaments extending substantially entirely across the mass, the filaments in the mass comprising a mixture of small-diameter filaments and comparatively large-diameter filaments heterogeneously distributed therethrough.

4. A low-density filamentous product comprising a bulky expanded mass of filaments exhibiting internal surfaces of cleavage, the strata comprising an irregular network of intercrossing filaments extending substantially entirely across the mass, the filaments in the mass comprising a mixture of solid filaments of small diameter and hollow filaments of larger diameter.

5. A low-density filamentous product comprising a bulky expanded mass of filaments exhibiting internal surfaces of cleavage, the strata comprising an irregular network of intercrossing filaments extending substantially entirely across the mass, the filaments in the mass comprising a mixture of solid filaments having an average diameter of about 1 to 10 microns and hollow filaments having an average diameter greater than 10 microns heterogeneously distributed therethrough.

6. A low-density filamentous product comprising a bulky expanded mass of filaments of a synthetic linear polymer, said mass exhibiting internal surfaces of cleavage, the strata comprising an irregular network of intercrossing filaments extending substantially entirely across the mass, the filaments in the mass comprising a mixture of small-diameter filaments and comparatively

large-diameter filaments heterogeneously distributed therethrough.

7. A low-density filamentous product comprising a bulky expanded mass of filaments of a synthetic linear polymer, said mass exhibiting internal surfaces of cleavage, the strata comprising an irregular network of intercrossing filaments extending substantially entirely across the mass, the filaments in the mass comprising a mixture of solid filaments having an average diameter of about 1 to 10 microns and hollow filaments having an average diameter greater than 10 microns heterogeneously distributed therethrough.

8. A low-density filamentous product comprising a bulky expanded mass having a specific gravity between 0.001 and 0.1 of filaments of a vinyl resin exhibiting internal surfaces of cleavage, the strata comprising an irregular network of intercrossing filaments extending substantially across the mass, the filaments in the mass comprising a mixture of solid filaments of small diameter and hollow filaments of larger diameter.

9. A low-density filamentous product comprising a bulky expanded mass having a specific gravity between 0.001 and 0.1 of filaments of a copolymer of vinyl acetate and vinyl chloride, said mass exhibiting internal surfaces of cleavage, the strata comprising an irregular network of intercrossing filaments extending substantially entirely across the mass, the filaments in the mass comprising a mixture of solid filaments having an average diameter of about 1 to 10 microns and hollow filaments having an average diameter of about 10 microns heterogeneously distributed therethrough.

10. A low-density filamentous product comprising a bulky expanded mass comprising a mixture of hollow filaments with solid filaments having an average diameter between 1 and 10 microns distributed therethrough, the bulk of the mass being constituted of the hollow filaments and a sufficient proportion of small filaments being present to impart a predetermined texture, stability, and impermeability to fluid.

11. A low-density filamentous product comprising a bulky expanded mass comprising a mixture of hollow filaments of a synthetic linear polymer with filaments of a synthetic linear polymer having an average diameter between 1 and 10 microns distributed therethrough, the bulk of the mass being constituted of the hollow filaments and a sufficient proportion of small filaments being present to impart a predetermined texture, stability, and impermeability to fluid.

12. A low-density filamentous product comprising a bulky expanded mass comprising a mixture of hollow hydrophobic vinyl resin filaments with hydrophobic vinyl resin filaments having an average diameter between 1 and 10 microns distributed therethrough, the bulk of the mass being constituted of the hollow filaments and a sufficient proportion of small filaments being present to impart a predetermined texture, stability, and impermeability to fluid.

13. A low-density filamentous product comprising a bulky expanded mass comprising a mixture of hollow filaments of a copolymer of vinyl chloride and vinyl acetate with filaments of a copolymer of vinyl chloride and vinyl acetate having an average diameter between 1 and 10 microns heterogeneously distributed therethrough, the bulk of the mass being constituted of the hollow filaments and a sufficient proportion of small filaments being present to impart a predetermined texture, stability and impermeability to fluid.